

Dec. 22, 1936.

J. I. BROBACK ET AL

2,065,045

CONSTRUCTION MATERIAL

Filed April 25, 1933



Fig. 1.



Fig. 2.



Fig. 3.



Fig. 4.



Fig. 5.



Fig. 6.

Inventors  
JUEL I. BROBACK AND  
GEORGE J. MARTIN,

By B. P. J. McElhenny

Attorney

## UNITED STATES PATENT OFFICE

2,065,045

## CONSTRUCTION MATERIAL

Juel Irvin Broback, Westfield, and George J.  
Martin, Denville, N. J.

Application April 25, 1933, Serial No. 667,922

3 Claims. (Cl. 20—91)

Our invention relates to a construction material which may be used as a substitute for ordinary wood.

An important object of the invention is to provide material of the above-mentioned character, which is capable of being cut and shaped by ordinary wood working tools, and is especially suited for the interior trim, partitions, ceilings, walls and floors of buildings, boats, etc.

10 A further object of the invention is to provide a material of the above-mentioned character, which is fire-proof or fire-retarding to a high degree.

15 A further object of the invention is to provide material of the above-mentioned character, which is water-resisting, to a high degree.

20 A further object of the invention is to provide a material of the above-mentioned character, which may be manufactured cheaply, and will not be materially heavier than ordinary lumber.

Other objects and advantages of the invention will be apparent during the course of the following description.

25 In the accompanying drawing, forming a part of this specification, and in which like numerals are employed to designate like parts throughout the same,

Figure 1 is a plan view of a section of material embodying our invention, parts being broken away in stepped relation, for the purpose of illustration,

Figure 2 is a vertical section taken on line 2—2 of Figure 1,

Figure 3 is an enlarged plan view of a portion 35 of the wire inserted asbestos fabric,

Figure 4 is a similar view of the asbestos fabric, without the wire insert,

Figure 5 is a vertical section through a modified form of the invention,

40 Figure 6 is a similar view through a further modified form of the invention.

In the drawing, wherein for the purpose of illustration are shown embodiments of our invention, attention being called first to Figures 1 to 3, 45 inclusive, the numeral 10 designates a core, of desired thickness. This core may be laminated, or it may be in one piece. The core may be formed of wood, paper, pulp, or other fibrous boards. As the material is designed to be used as a fire- 50 proof or fire-retarding medium, satisfactory re-

sults are obtained by forming the core of alternate sections or strips of wood 11 and 12. The strips 11 may be of basswood, and the strips 12 of birch wood. These strips are securely glued together at their edges. The invention is in no sense restricted to the employment of this precise material, nor is the invention necessarily restricted to the laminated character of the core. The laminated character of the core, however, aids in preventing warping of the completed 10 board, as when subjected to the action of high heat.

A layer of woven asbestos fabric 14 is placed upon each layer 13. This woven asbestos fabric is radically different in construction, and function, from asbestos paper or felt. Woven asbestos fabric consists of strands of asbestos woven to produce a cloth or fabric. Woven asbestos fabric has superior fire-resisting qualities, superior tensile strength, minimum weight, and effects a perfect bond between the laminations through the medium of a binder, such as water-proof glue. The strength of the woven asbestos fabric permits the laminations being securely bonded together. The woven asbestos fabric embodies 25 threads or yarns having a high asbestos content. The woven asbestos fabric has an asbestos content of about 90% pure asbestos fibre. The use of the woven asbestos fabric increases the weight of the final product only about 10%, while impregnated fire-proof wood increases the weight from 25% to 40%, depending on the degree of fire-proofness. Asbestos paper contains only about 20% of pure asbestos fibre. Asbestos paper is stratified and has a low tensile strength and 30 readily splits or separates into layers, and therefore cannot make a strong bond between the laminations. Asbestos paper also has a lower fire-resistance. The asbestos fabric 14 has its strands 14 provided with wire inserts 14<sup>a</sup>, preferably formed of fine plated brass strands, about which the asbestos yarn is wound. We also contemplate using an asbestos fabric 14, Figure 4, wherein the wire 14<sup>a</sup> is omitted.

The laminations in Figure 1 are shown as applied to both sides of the core 10, but some degree of success may be had by applying them to one side only.

An outer layer 15 is provided, which may be formed of wood veneer, paper, pulp, or other 50

fibrous material. If the layers 13 and 15 are formed of wood, their grains are arranged at a right angle. In one specimen which we made, one layer 15 was walnut veneer and the other layer 15, maple.

- 5 In assembling the various layers, the surfaces of the core 10 are coated with a water-proof glue, the surfaces of the cross bands 13 are also coated with water-proof glue, the surfaces of the woven asbestos fabric 14 are coated with this water-proof glue, and the interior surfaces of the outer layers 15 are coated with this water-proof glue. These superposed layers, when assembled, are subjected to a pressure of about 100 pounds per 10 square inch, and the glue is allowed to dry under this pressure. The glue may be applied to the laminations by means of a glue spreader, consisting of two rollers receiving glue thereon, between which the said lamination is run.
- 15 20 While it is preferred to use the cross bands 13, they may be omitted, as shown in Figure 5, in which event the woven asbestos fabric will be directly cemented upon the core 10. When the word "core" is used in the claims, without additional limitations, it is intended that this word cover the inner element including the strips 11, without the bands or veneer 13, Figure 5, or an inner element including the strips 11 and bands or veneer 13.

- 25 30 In Figure 6, we have shown a further modification of the invention, wherein the woven asbestos fabric 14 is employed and is arranged between two strips or sheets 16, and is glued or cemented thereto. These strips or sheets may be formed 35 of wood, paper pulp, or other fibrous material. In this form of the invention, the core 10 is omitted.

40 The water-proof glue which we prefer to use has a glue mineral base, and when dry is a rock-like material which is not only water-proof but fireproof. This glue contains casein, which is a mineral. The invention is not restricted to the use of this particular type of glue, as other glues or cements may be employed. Further, the laminations may be secured together by means other than glue. They may be secured together by 45 nails, screws, or the like.

50 A specimen embodying a preferred embodiment of the invention, as described in Figures 1 to 4, inclusive, the wire not being present in the asbestos woven fabric, was subjected to a fire test. The flame from an air-gas torch was applied to the walnut-veneered surface, and the effect upon the specimen recorded in the log of 55 fire test.

60 The temperature at the point of application of the flame and on the underside of the specimen were recorded with a Leeds and Northrup potentiometer temperature indicator. The temperature was raised to 1700° F. in thirty minutes, and maintained for thirty minutes at 1700° F. At the end of the test the specimen was submerged in water and the effect upon the specimen noted.

65 The following log of test gives the data recorded during the test:

| Time<br>minutes | Temperature of<br>flame |               | Remarks                                                                                                     | 5  |
|-----------------|-------------------------|---------------|-------------------------------------------------------------------------------------------------------------|----|
|                 | Top<br>side             | Under<br>side |                                                                                                             |    |
| 0               | ° F.<br>70<br>900       | ° F.<br>70    | Room temperature 70° F.                                                                                     |    |
| 3               |                         |               | Wood began charring. Charred area, diameter=1 inch.                                                         |    |
| 7               | 1040                    | 70            | Charred area increasing slowly. No flaming on removal of flame.                                             | 10 |
| 12              | 1140                    | 74            | Charred area increased to 2 inches diameter.                                                                |    |
| 15              | 1220                    | 84            | Charred area, diameter=2 inches.                                                                            |    |
| 17              | 1240                    | 92            | Layer of asbestos becoming exposed.                                                                         |    |
| 21              | 1240                    | 98            |                                                                                                             |    |
| 23              | 1470                    | 106           | Flaming in spots on removal of flame. Top layer of walnut veneer charred, exposing asbestos layer.          | 15 |
| 27              | 1400                    | 117           |                                                                                                             |    |
| 30              | 1480                    | 124           | Charred area, 3 inches in diameter.                                                                         |    |
| 33              | 1675                    | 134           | Veneer flaming slightly on removal of flame. Asbestos glowing under flame, glow fading on removal of flame. |    |
| 37              | 1730                    | 150           | Charred area, 5 inches in diameter.                                                                         | 20 |
| 40              | 1650                    | 170           |                                                                                                             |    |
| 42              | 1730                    | 190           | Asbestos glowing, but shows no signs of breaking up.                                                        |    |
| 44              | 1700                    | 204           |                                                                                                             |    |
| 50              | 1740                    | 262           | Charred area, 6 inches in diameter. Asbestos showing signs of breaking up.                                  |    |
| 57              | 1700                    | 280           | No signs of charring on underside.                                                                          | 25 |
| 60              | 1700                    | 290           | Signs of charring and cracking of veneer on under side. No change after application of water.               |    |

30 Although the surface appeared charred it seemed intact, but the asbestos and wood core was easily scraped away indicating oxidation of the material.

35 After removing charred portion, an opening 4 inches in diameter was formed, extending through the basswood and birch core, which was charred and cracked. The opening on the underside was about  $\frac{1}{2}$  inch in diameter.

40 Having fully described our invention, what we claim is:

45 1. A building material comprising layers of fibrous material and a layer of woven asbestos fabric between said layers, said fabric comprising strands having wire inserts, said layers being securely cemented together.

50 2. A fire resisting building board, comprising a core, said core including strips of wood having their edges cemented together, sheets of wood veneer cemented to the opposite faces of the core, sheets of fire resisting fabric cemented to the outer faces of the sheets of veneer, said fire resisting fabric including woven metal strands having a covering of asbestos yarn wound thereon, and sheets of veneer cemented to the outer faces of the fire resisting fabric.

55 3. A building board comprising a core, sheets of fire resisting fabric arranged upon the opposite faces of the core, said fabric comprising woven wire strands having a covering of asbestos yarn wound thereon, and a water-proof glue containing casein for securely binding these elements together and producing a rock-like material when dry which is fire-proof.

60 JUEL IRVIN BROBACK.  
GEORGE J. MARTIN. 65